# EUROPEAN PATENT APPLICATION

(11) **EP 3 786 354 A1**
(43) Date of publication of application: **03.03.2021**
(21) Application number: 18917014.5
(22) Date of filing: 06.07.2018
(51) Int. Cl.: D06P 1/00, D06P 1/94, D06P 1/16, D06P 3/54, D06P 1/38, D06P 3/66, D06P 5/02, D06B 9/02, D06B 9/06

(54) **SUPERCRITICAL CODYEING METHOD AND DYEING SYSTEM**

(30) Priority: 27.04.2018 CN 201810394114
(71) Applicant: Qingdao Jifa Group Co., Ltd., Shandong 266200 (CN)
(72) Inventor: WANG, Jian, Qingdao, Shandong 266200 (CN); YANG, Weidong, Qingdao, Shandong 266200 (CN); WAN, Gang, Qingdao, Shandong 266200 (CN); LIU, Chongbo, Qingdao, Shandong 266200 (CN); LIU, Shaobing, Qingdao, Shandong 266200 (CN); LIN, Dapeng, Qingdao, Shandong 266200 (CN); WANG, Dawei, Qingdao, Shandong 266200 (CN); DAI, Zhijing, Qingdao, Shandong 266200 (CN)
(74) Representative: Høiberg P/S
(86) International application number: PCT/CN2018/094762
(87) International publication number: WO 2019/205297

(57) **Abstract**

A supercritical CO 2 dyeing method and a dyeing system. The dyeing method comprises the following steps: S1, dyeing: placing an object to be dyed on a staining system to complete a dye adsorption process; S2, color fixation in a supercritical CO 2 dynamic color fixation system: placing the object to be dyed which is stained in step S1 into a dyeing curing kettle, starting a pressurizing pump, pumping an appropriate amount of CO 2, enabling the CO 2 in the dyeing curing kettle to reach a supercritical state, heating the dyeing curing kettle, when the temperature and pressure in the dyeing curing kettle reach a process parameter setting value, starting a circulating pump, enabling the supercritical CO 2 fluid of the supercritical CO 2 dynamic color fixation system to be slowly circulated, and after a period of time, completing the dye/pigment diffusion and fixation process on the object to be dyed in the dyeing curing kettle; and S3, releasing the pressure, and separating the CO 2. The dyeing method and the dyeing system have the advantages of high production efficiency, uniformity in dye fixation, material conservation and wide dye application range, and are suitable for dyeing various fiber fabrics.

## Description

### Technical field

The invention belongs to the technical field of dyeing, and relates to supercritical CO₂ waterless dyeing or dyeing without water technology, in particular to a supercritical CO2 dyeing method and a dyeing system.

### Background

In conventional textile dyeing, large amounts of water are used as medium to drain out sewage containing chemicals, such as dyes and surfactants, which are harmful to the sustainable development of the environment. In most regions of China, the shortage of water, especially due to the discharge of sewage, has become a severe issue in recent years and is the key factor imposing restrictions on the development of the textile dyeing and finishing industry. In order to prevent pollution, research on green and effective dyeing process is seen as one that will steer the industry in the right direction.

Supercritical CO₂ waterless dyeing is a new type of green dyeing method, which has characteristics of high efficiency, no pollution and much shorter in dyeing time. In its dyeing process, supercritical CO₂ is used as the dyeing medium and carbon dioxide turns to a supercritical state, neither a complete gas state nor a liquid state, at a pressure higher than 7.3MPa and a temperature higher than 31°C. In the prior art, most of the supercritical fluid is pressed by a circulation pump to circulate continuously between dye caldron and dyeing caldron; during the movement carbon dioxide works as a carrier to transfer the dissolved dye to pores in fibers so as to achieve color with desired uniformity in a short time, (such as Chinese Patent: CN106757915A). The dyeing process does not require procedures as washing or drying. Many countries are striving to develop such new green energy-saving dyeing and finishing device and try to make it industrialization and into practical use.

In the prior art, the process of supercritical CO₂ waterless dyeing can be divided into four stages: dye dissolution, adsorption, diffusion and fixation. Dyes are placed in the dye caldron, and the supercritical fluid flows through the dye caldron to dissolve dyes (such as Chinese patent: CN206015309U), and then the solution which carries the dissolved dyes flows through the object to be colored; after a period of time, the fixation process completes and the solution flows into recovery caldron for separation and recovery. However, currently there are only a few dyes could be dissolved in supercritical CO₂ and merely polyester could be dyed, which restricts the industrialization and scale development of supercritical dyeing.

Chinese patent (CN102817194B) discloses a static dyeing method and a device using the same with supercritical fluid, in which the object to be dyed is stained by immersion at first and then placed in a supercritical fluid. However it has some problems: 1. dye migration may occur by immersion to cause uneven fabric dye; 2. only for polyester it is a physical process, but for fibers such as cotton and nylon it will lead to chemical changes so could not be used; 3. the static dyeing requires varied process parameters in different positions of the system which will result in obvious color deviation thereon.

In view of the development and drawbacks of the conventional supercritical CO₂ waterless dyeing processes hereinabove described, how to provide with a supercritical CO₂ dyeing technology involving a dying and curing process route and a device for achieving the same applicable to natural fibers, chemical fibers and blended fibers is an urgent requirement for the industry.

### Summary

In order to solve the above problems and deficiencies in the prior art, the present invention provides a supercritical CO₂ dyeing method and a dyeing system, which have the advantages of high in production efficient, good in uniformity, saving in material and applicable to a wide range of dyes or pigments. The supercritical CO₂ dyeing method and a dyeing system could be used for dyeing and curing natural fibers, chemical fibers and blended fibers.

The object of the present invention is achieved by the following technical solutions:
A supercritical CO₂ dyeing method, characterized in that the dyeing method comprises:
S1: dyeing: enabling an object to be dyed to complete a dye/pigment adsorption process in a coloring assembly, in which dyes or pigments used are insoluble in CO₂;
S2: fixing with a supercritical CO₂ fluid fixation assembly: putting the object to be dyed which is colored in the Step S1 into a dyeing and curing kettle; turning on a pressure pump to pump into a proper amount of CO₂ into the supercritical CO₂ fluid fixation assembly; enabling the CO₂ in the dyeing and curing kettle to reach to a supercritical state; heating the dyeing and curing kettle; when the temperature and pressure inside the dyeing and curing kettle reaches to values of preset process parameters, a circulation pump is turned on to enable the supercritical CO₂ fluid in the supercritical CO₂ fluid fixation assembly to slowly circulate for a period of time; when the period of time expires, a dye/pigment diffusion and fixation process of the object to be dyed within the dyeing and curing kettle is completed;
S3: when the fixation process is completed, a pressure relief valve is opened to relieve and the CO₂ fluid flows into a recovery kettle to separate and recover CO₂.

Further: after the Step S3, opening the dyeing and curing kettle and taking out the object to be dyed after the fixation to wash or soap.

Further the object to be dyed is textiles; in the Step S1, the object to be dyed is colored by means of immersion or sizing which includes: preparing a desired dyeing precursor in which one or more suitable auxiliary agents are added into for improving the uniformity of adhesion, or preparing coating slurry according to different fabric materials; in the Step S2, fabrics are placed into the supercritical fluid in the dyeing and curing kettle by means of a warp beam, preset process parameters includes: a pressure for fixation is 8MPa-30MPa, a temperature is 60°C to 150°C, a volume of fluid circulation in the supercritical CO₂ fluid dynamic fixation assembly is 100-1000L/h and a cycle of the dyeing process is 10min-120min; and one or more catalysts are added during the curing process in the Step S2 to make dyes/pigments to penetrate through the fabric fibers more uniformly and deeply.

Further, the object to be dyed is polyester fabrics and disperse dyes are used as dyestuffs;
the Step S1 includes: adding an appropriate amount of one or more suitable thickening auxiliary agents to a dyeing precursor, immersing the polyester fabrics by means of a rolling mill, enabling the polyester fabrics to pass through the prepared precursor at a constant speed and squeezing the polyester fabrics, which is tensioned by rollers, by squeeze wheels, wherein the ratio of the dyeing precursor contained in the polyester fabrics is controlled by adjusting the pressure exerted by the squeeze wheels to 0-0.8MPa; the Step S2 includes: loading the bathed polyester fabrics on the dyeing warp beam and putting the polyester fabrics into the dyeing and curing kettle, opening the pressure pump to pump into an appropriate amount of CO₂ into the circulation, turning on the heating jackets and the heat trace cables to heat the dyeing and curing kettle; when the temperature in the circulation reaches 80-140°C and the pressure reaches to 8-27 MPa which are the values of preset process parameters, turning on the circulation pump at a flow rate≥20L/h; after a period of time of 10-40 min, the dye diffusion and fixation process on the polyester fabrics is completed.

Further: the object to be dyed is polyester fabrics and a method of pigment sizing is adopted to cover the polyester fabrics in the step S1; the step S1 includes: preparing suitable coating slurry, in which one or more adhesives are added into for fixation of the slurry; enabling the polyester fabrics to pass through a coating machine or a printing machine so as to uniformly apply the slurry to the polyester fabrics; the step S2 includes: loading the immersed polyester fabrics on the dyeing warp beam and putting the polyester fabrics into the dyeing and curing kettle, opening the pressure pump to pump into an appropriate amount of CO₂ into the supercritical CO₂ fluid fixation assembly, turning on the heating jackets and the heat trace cables to heat the dyeing and curing kettle; when the temperature in the supercritical CO₂ fluid fixation assembly reaches 80-140°C and the pressure reaches to 8-27 MPa which are the values of preset process parameters, turning on the circulation pump at a flow rate≥20L/h; after a period of time of 10-40 min, the dye diffusion and fixation process on the polyester fabrics is completed.

Further, when the object to be dyed is cotton fabrics, in the Step S2, the humidity within the supercritical CO₂ fluid dynamic fixation assembly is controlled between 40% and 90% and urea is added as a wetting agent to ensure the humidity during the curing process.

Further, the object to be dyed is textiles made of natural fibers, chemical fibers or blended fibers or textile articles, and dyes is at least one dyestuff selected from the group consisting of direct dyes, reactive dyes, cationic dyes, disperse dyes, vat dyes, azo dyes and sulfur dyes.

A dyeing system for the supercritical CO₂ dyeing method according to any one of claims 1-7, characterized in that the dyeing system comprises: a coloring assembly including rolling mill, a coating machine or a printing machine; and a supercritical CO₂ fluid fixation assembly, which is a supercritical CO₂ fluid dynamic fixation assembly, including: a dyeing and curing kettle, a recovery kettle, a circulation connecting the dyeing and curing kettle and the recovery kettle, which comprises a CO₂ gas cylinder, a pressure pump, a circulation pump and pipelines thereamong, wherein the pressure pump and a valve III are disposed on a pipeline from the outlet of the CO₂ gas cylinder, and the outlet of the valve III is respectively connected to the outlet of the dyeing and curing kettle and the outlet of the recovery kettle in two ways; the circulation pump and a valve I are disposed on a pipeline connecting the outlet of the dyeing and curing kettle and the inlet of the recovery kettle, a pressure relief valve, which is disposed on a pipeline connecting the outlet of the dyeing and curing kettle and the inlet of the recovery kettle, a valve II, which is disposed on a pipeline connecting the outlet of the CO₂ gas cylinder and the outlet of the recovery kettle; heating jackets, which are disposed out of the dyeing and curing kettle and the recovery kettle, and heat trace cables, which are wound around the pipelines connected to the dyeing and curing kettle and the recovery kettle.

Further: the dyeing and curing kettle has a horizontal cylindrical kettle body and the recovery kettle has an elongated cylindrical kettle body in which a three-dimensional duplex filter structure is disposed.

Further wherein the coating machine employs a classic coating machine or a foam coating machine; the printing machine employs a cylinder printing machine, a flat screen printing machine or an ink jet printing machine.

### Beneficial effect

Compared with the prior art, the invention has the following advantages and positive effects:
1. Since the dyeing process of the present invention could use those water-soluble dyes, the process is completely free from the limitation that only a few available dyes (supercritical CO₂ soluble dyes) could be used in the conventional supercritical CO₂ dyeing, the selection of dyestuffs is more abundant to satisfy the requirements of production.
2. Since most of the water-soluble dyes could not be dissolved in supercritical CO₂, the color on the fabrics after supercritical CO₂ fixation is uniform without color shading as long as the dyes or pigments uniformly dyed during rolling or sizing, which is comparatively easy to operate.
3. The invention adopts supercritical CO2 fluid dynamic curing throughout the curing process, in which each position can meet the requirements of the process parameters, thereby accelerating the diffusion rate of the dyes in the system and improving the fixing rate.
4. The invention could ensure a thorough fixation of color. Coated fabrics are currently cured by hot air or saturated steam, by which coating usually only forming on the surface instead of inside the fibers. The invention adopts supercritical CO₂ to cure fibers and the microscopic detection shows that the dyestuffs can enter into the interior of the fibers, namely enable them to be completely dyed.
5. The invention has high production efficiency. The fabrics is loaded in the supercritical CO₂ fluid by means of a warp beam which occupied a very small space and the time period for curing is same as that of the conventional fixation process.
6. The supercritical CO₂ dynamic fixation system of the present invention is free from the dependence of traditional medium water in dyeing and 90% of CO₂ could be recycled. The present invention is a solution to the production and discharge of pollutants from the source and has the characteristics of environmental-friendly and green, which could be widely applied to the energy saving, emission reduction and clean production in prospect in the textile printing and dyeing industry.

### Brief Description of Drawings

Fig.1 is a schematic structural view of a supercritical CO₂ fluid dynamic fixation assembly according to the present invention;
Fig.2 is a schematic view showing a process route of a supercritical CO2 dyeing method of the present invention;
Fig. 3 is a photomicrograph of a polyester fiber fixed by a conventional dyeing process;
Fig. 4 is a photomicrograph of a polyester fiber fixed by a supercritical CO₂ dyeing method according to the present invention.

In the drawings, 1-valve I; 2-dyeing and curing kettle; 3-recovery kettle; 4-valve II; 5-CO₂ gas cylinder; 6-pressure relief valve; 7-pressure pump; 8-valve III; 9-Circulation pump.

### Detailed Description of the Embodiments

Referring to Fig. 1 and Fig.2, a supercritical CO₂ dyeing method and a system for supercritical CO₂ dyeing are disclosed. The system for supercritical CO₂ dyeing includes a coloring assembly and a supercritical CO₂ fluid fixation assembly, wherein the coloring assembly includes a rolling mill, a coating machine or a printing machine; the supercritical CO₂ fluid fixation assembly is a supercritical CO₂ fluid dynamic fixation assembly. The supercritical CO₂ fluid dynamic fixation assembly comprises a dyeing and curing kettle 2, a recovery kettle 3 and a circulation connecting the dyeing and curing kettle 2 and the recovery kettle 3, wherein the circulation comprising a CO₂ gas cylinder 5, a pressure pump 7, a circulation pump 9 and pipelines thereamong. The pressure pump 7 and a valve III 8 are disposed on a pipeline from the outlet of the CO₂ gas cylinder 5, and the outlet of the valve III 8 is respectively connected to the outlet of the dyeing and curing kettle 2 and the outlet of the recovery kettle 3 in two ways. The circulation pump 9 and a valve I 1 are disposed on a pipeline connecting the outlet of the dyeing and curing kettle 2 and the inlet of the recovery kettle 3. A pressure relief valve 6 is disposed on a pipeline connecting the outlet of the dyeing and curing kettle 2 and the inlet of the recovery kettle 3. A valve II 4 is disposed on a pipeline connecting the outlet of the CO₂ gas cylinder 5 and the outlet of the recovery kettle 3. Heating jackets are disposed out of the dyeing and curing kettle 2 and the recovery kettle 3 and heat trace cables are wound around the pipelines connected to the dyeing and curing kettle 2 and the recovery kettle 3.

Preferably, the dyeing and curing kettle 2 has a horizontal cylindrical kettle body and the recovery kettle 3 has an elongated cylindrical kettle body in which a three-dimensional duplex filter structure is disposed.

Preferably, the coating machine employs a classic coating machine well known to one skilled in the art or a foam coating machine; the printing machine employs a cylinder printing machine, a flat screen printing machine or an ink jet printing machine.

Since the supercritical CO₂ fluid in the dyeing and curing kettle 2 and the recovery kettle 3 are going to work in a high temperature and high pressure state, those valves mentioned above are high pressure and high temperature valves.

When the supercritical CO₂ fluid dynamic fixation assembly is in a working state, the valve I 1, the valve II 4 and the valve III 8 are open and the pressure relief valve 6 is closed until a curing process ends, and thereafter the pressure relief valve 6 is opened to relieve the system the CO₂ flows into the recovery kettle 3 for separation and recycle.

Referring to Fig. 1 and Fig.2, a supercritical CO2 dyeing method is disclosed based on the system for supercritical CO₂ dyeing disclosed above, which includes the following steps:
S1: dyeing: enabling the object to be dyed to complete a dye/pigment adsorption process in the coloring assembly; the dye or pigment used is insoluble in CO₂;
S2: fixing with the supercritical CO₂ fluid dynamic fixation assembly: putting the object to be dyed which is colored in the step S1 into the dyeing and curing kettle 2; turning on the pressure pump 7 to pump into a proper amount of CO₂; enabling the CO₂ in the dyeing and curing kettle 2 to reach to its supercritical state; heating the dyeing and curing kettle 2. When the temperature and pressure in the dyeing and curing kettle 2 reaches to values of preset process parameters, the circulation pump 9 is turned on to enable the supercritical CO₂ fluid in the supercritical CO₂ fluid dynamic fixation assembly to slowly circulate for a period of time; when the period of time expires, the dye/pigment diffusion and fixation process of the object to be dyed within the dyeing and curing kettle 2 is completed.
S3: When the fixation process is completed, the pressure relief valve 6 is opened to relieve the system, and the CO₂ fluid flows into the recovery kettle 3 to separate and recover CO₂.

After the completion of the step S3, the step S4 is further performed: the dyeing and curing kettle 2 is opened and the object to be dyed after the fixation is taken out, and thereafter to be washed or soaped.

Specifically, the above-mentioned object to be dyed is fabrics; in the Step S1, the object is colored by means of immersion or sizing which includes preparing a desired dyeing precursor in which one or more suitable auxiliary agents are added into for improving the uniformity of adhesion, or preparing coating slurry according to different fabric materials; in the Step S2, fabrics are placed into the supercritical fluid in the dyeing and curing kettle 2 by means of a warp beam, the preset process parameters includes: the pressure for fixation is 8MPa-30MPa, the temperature is 60°C to 150°C, the volume of fluid circulation in the supercritical CO₂ fluid dynamic fixation assembly is 100-IOOOL/h and the cycle of the dyeing process circulation is 10min-120min.

The process of the invention is further illustrated by the following examples.

Example 1: the object to be dyed is polyester fabrics and disperse dyes are used as dyestuffs; in the Step S1, adding an appropriate amount of one or more suitable thickening auxiliary agents to a dyeing precursor, immersing the polyester fabrics by means of a rolling mill, enabling the polyester fabrics to pass through the prepared precursor at a constant speed and squeezing the polyester fabrics, which is tensioned by one or more rollers, by one or more squeeze wheels, wherein the ratio of the dyeing precursor contained in the polyester fabrics is controlled by adjusting the pressure exerted by the squeeze wheels so as to control the shade of color on the polyester fabrics; in the Step S2, loading the bathed polyester fabrics on the dyeing warp beam and putting the polyester fabrics into the dyeing and curing kettle 2, closing the valves, opening the pressure pump to pump into an appropriate amount of CO₂ into the circulation, turning on the heating jackets and the heat trace cables to heat the dyeing and curing kettle 2; when the temperature in the circulation reaches 80-140 °C and the pressure reaches to 8-27 MPa which are the values of preset process parameters, turning on the circulation pump 9 at a flow rate≥20L/h. After a period of time of 10-40 min, the dye diffusion and fixation process on the polyester fabrics is completed. Preferably, when controlling the ratio of the dyeing precursor contained in polyester fabric by adjusting the pressure of the squeeze wheel, the pressure applied to the fabric ranges from 0 to 0.6 MPa.

Example 2, the object to be dyed is polyester fabrics and the method of pigment sizing is adopted to cover the polyester fabrics in the step S1; the Step S1 includes: (1) preparing suitable coating slurry, in which one or more adhesives are added into for fixation of the slurry; (2) enabling the polyester fabrics to pass through a coating machine or a printing machine so as to uniformly apply the slurry to the polyester fabrics; the Step S2 includes, loading the immersed polyester fabrics on the dyeing warp beam and putting the polyester fabrics into the dyeing and curing kettle 2, opening the pressure pump to pump into an appropriate amount of CO₂ into the supercritical CO₂ fluid dynamic fixation assembly, turning on the heating jackets and the heat trace cables to heat the dyeing and curing kettle 2; when the temperature in the circulation reaches 80-140°C and the pressure reaches to 8-27 MPa which are the values of preset process parameters, turning on the circulation pump 9 at a flow rate ≥20L/h. After a period of time of 10-40 min, the dye diffusion and fixation process on the polyester fabrics is completed.

Referring to Fig.3 and Fig. 4, a photomicrograph of a supercritical cured polyester fiber produced by the dyeing method or the system according to the present invention and a photomicrograph of cured polyester fiber produced by a conventional dyeing process are compared. In the conventional way, coated fabrics are cured by heated air or saturated steam so that the coatings are merely cured onto the surfaces of fabrics instead of entering the interior of the fiber (shown in Fig. 3), while the microscopic detection of the polyester fiber cured by supercritical CO₂ according to the present invention shows that the dyestuffs could enter into the interior of the polyester fiber to make it completely dyed (shown in Fig. 4).

When the object to be dyed is cotton fabrics, in the Step S2, the humidity within the supercritical CO₂ fluid dynamic fixation assembly should be controlled between 40% and 90% and urea is added as a wetting agent to ensure the humidity during the curing process.

Preferably, fabrics are wrapped around the dyeing warp beam and the dyeing and curing kettle 2 is arranged in a horizontal manner so that the occupied space is very small and the duration of the curing process is same as that of the conventional process, which is high in efficiency.

In order to increase the rate of curing of dyes which is insoluble in the supercritical fluid onto fabrics, one or more suitable catalysts are added during the curing process in the Step S2 to make dyes/pigments to penetrate through the fabric fibers more uniformly and deeply.

The object to be dyed mentioned in the present invention could be fabrics made of natural fibers, chemical fibers or blended fibers or other textile articles. The textile articles include garment products, shoes, hats, accessories and the like. The fabrics include textiles made of pure polyester knitted fabrics, pure polyester woven fabrics or cotton fabrics, and also include other yarn interwoven fabrics or composite fabrics. The garment products include knitted underwear, shirts, sportswear, uniforms, skirts, jackets, suits and the like. Accessories include ties, scarves and the like.

Dyes used in the supercritical CO₂ dyeing method of the present invention could be at least one dyestuff selected from the group consisting of direct dyes, reactive dyes, cationic dyes, disperse dyes, vat dyes, azo dyes and sulfur dyes.

It should be emphasized that the key to the method or the system disclosed by the present invention is that the fixation is done in the supercritical CO₂ dynamic fixation assembly and the dye/pigment used is insoluble in CO₂. The process for coloring can adopt those typical procedures well known to one skilled in the art, where classic dyeing equipment is used. For example, the coating machine could employ a classic coating machine or a foam coating machine; and the printing machine could employ a cylinder printing machine, a flat screen printing machine or an ink jet printing machine, even hand-painting or printing could be used for coloring.

Specific examples of the supercritical CO₂ dyeing method are described as follows:
Specific Example 1: polyester fabrics are dyed with disperse dyes insoluble in CO₂.
1. According to preset dyeing process requirements, an appropriate amount of disperse dyes is dissolved in water in which a suitable amount of one or more thickening auxiliary agents are added into the water to improve the adsorption capability of the dye precursor onto polyester yarns. Polyester fabrics pass through the pre-formed dye precursor, and thereafter are tensioned by rollers of a rolling mill and squeezed by pressing wheels, wherein the pressure exerted by the pressing wheels is adjusted to 0.1MPa.
2. Polyester fabrics immersed are wound on a dyeing warp beam and placed in the dyeing and curing kettle 2. The pressure pump 7 is turned on to pump into an appropriate amount of CO₂ into the supercritical CO₂ fluid dynamic fixation assembly and the heating jackets and the heat trace cables are activated. When the temperature in the supercritical CO₂ fluid dynamic fixation assembly reaches to 85 °C and the pressure therein reaches to 10MPa which are the values of preset process parameters, the circulation pump 9 is turned on. After a period of time of 40min, the recovery procedure starts by opening the pressure relief valve 6, the fluid flows into the recovery kettle 3 for the separation and recycle of CO₂. The curing process is completed.

Specific Example 2: polyester fabrics are dyed with disperse dyes insoluble in CO₂.
1. According to preset dyeing process requirements, an appropriate amount of disperse dye is dissolved in water in which a suitable amount of one or more thickening auxiliary agents are added into water to improve the adsorption capability of the dye precursor onto the polyester yarns. Polyester fabrics pass through the pre-formed dye precursor, and thereafter are tensioned by rollers of the rolling mill and squeezed by pressing wheels, wherein the pressure exerted by the pressing wheel is adjusted to 0.6MPa.
2. Polyester fabrics immersed are wound on a dyeing warp beam and placed in the dyeing and curing kettle 2. The pressure pump 7 is turned on to pump into an appropriate amount of CO₂ into the supercritical CO₂ fluid dynamic fixation assembly and the heating jackets and the heat trace cables are activated. When the temperature in the circulation reaches to 120°C and the pressure therein reaches to 27MPa which are the values of preset process parameters, the circulation pump 9 is turned on. After a period of time of 10min, the recovery procedure starts by opening the pressure relief valve 6, the fluid flows into the recovery kettle 3 for separation and recycle CO₂. The curing process is completed.

Test results of performance indicators of the printing and curing process in Specific Example 1 and Specific Example 2:
Based on *China Natiaonal Standard: GB*/*T 3921.1-1997 Textiles-Tests for color fastness-Color fastness to washing: Test 1, GB7565-87 Textiles-Tests for color fastness- Specification for standard adjacent fabric: Cotton and viscose* and *GB6151-857Textiles-Tests for color fastness-General principle of testing*, color fastness of fabrics dyed by the two above-mentioned specific examples is evaluated and the results show that the rubbing fastness and wash fastness of the both of the dyed fabrics meets the requirements of *GB 18401-2003 National general safety technical code for textile products*, wherein the rubbing fastness could reach Grade 3 and above and the washing fastness could reach Grade 4 and above.

Specific Example 3: cotton fabrics are dyed with reactive dyes.
1. According to preset dyeing process requirements, an appropriate amount of reactive dyes is dissolved in water in which Na₂CO₃ is added into to adjust the pH of the dyeing solution alkaline and urea is added into as a wetting agent. Cotton fabrics pass through the pre-formed dyeing precursor at a constant speed, and thereafter are tensioned by rollers of a rolling mill and squeezed by pressing wheels, wherein the pressure exerted by the pressing wheels is adjusted to 0.4MPa.
2. Cotton fabrics immersed is wound on a dyeing warp beam and placed in the dyeing and curing kettle 2. The pressure pump 7 is turned on to pump into an appropriate amount of CO₂ into the supercritical CO₂ fluid dynamic fixation assembly and the heating jackets and the heat trace cables are activated. When the temperature in the circulation reaches to 120°C and the pressure reaches to 27MPa which are the values of preset process parameters, the circulation pump 9 is turned on. After a period of time of 10min, the recovery procedure starts by opening the pressure relief valve 6, the fluid flows into the recovery kettle 3 for separation and recycle of CO₂. The curing process is completed.

### Specific Example 4: curing of flat screen printing fabrics

1. According to preset dyeing process requirements, a color paste with suitable viscosity and consistency is prepared, a printing machine pastes the fabrics on a straight and seamless annular guide belt running along the warp direction where the fabrics intermittently runs with the guide belt. A color frame is fixed above the fabrics and makes an up-down movement. When the guide belt is stationary, the color frame is lowered to enable a squeegee to reciprocate for pressing and scratching the color paste to make the color paste through a mesh and be printed on the fabrics.
2. Fabrics immersed is wound on a dyeing warp beam and placed in the dyeing and curing kettle 2. The pressure pump 7 is turned on to pump into an appropriate amount of CO₂ into the supercritical CO₂ fluid dynamic fixation assembly and the heating jackets and the heat trace cables are activated. When the temperature in the circulation reaches to 120°C and the pressure reaches to 25MPa which are the values of preset process parameters, the circulation pump 9 is turned on. After a period of time of 10min, the recovery procedure starts by opening the pressure relief valve 6, the fluid flows into the recovery kettle 3 for separation and recycle of CO₂. The curing process is completed.

Test results of performance indicators of the printing and curing process in Specific Example 3 and Specific Example 4:
Based on *China Natiaonal Standard: GB*/*T 3921.1-1997 Textiles-Tests for color fastness-Color fastness to washing: Test 1*, *GB7565-87 Textiles-Tests for color fastness- Specification for standard adjacent fabric: Cotton and viscose* and *GB6151-857Textiles-Tests for color fastness-General principle of testing,* color fastness of fabrics dyed by the two above-mentioned specific examples is evaluated and the results show that the rubbing fastness and wash fastness of the both of the dyed fabrics meets the requirements of *GB 18401-2003 National general safety technical code for textile products*, wherein the rubbing fastness could reach Grade 3-4 to and the washing fastness could reach Grade 4-5.

The above description is not intended to limit the invention, and the invention is not limited to the above examples, and variations, modifications, additions or substitutions made by those skilled in the art within the scope of the invention are also It should fall within the scope of protection of the present invention.

## Claims

1. A supercritical CO₂ dyeing method, **characterized in that** the dyeing method comprises:
S1: dyeing: enabling an object to be dyed to complete a dye/pigment adsorption process in a coloring assembly, in which dyes or pigments used are insoluble in CO₂;
S2: fixing with a supercritical CO₂ fluid fixation assembly: putting the object to be dyed which is colored in the step S1 into a dyeing and curing kettle (2); turning on a pressure pump (7) to pump into a proper amount of CO₂ into the supercritical CO₂ fluid fixation assembly; enabling the CO₂ in the dyeing and curing kettle (2) to reach to a supercritical state; heating the dyeing and curing kettle (2); when the temperature and pressure inside the dyeing and curing kettle (2) reaches to values of preset process parameters, a circulation pump (9) is turned on to enable the supercritical CO₂ fluid in the supercritical CO₂ fluid fixation assembly to slowly circulate for a period of time; when the period of time expires, a dye/pigment diffusion and fixation process of the object to be dyed within the dyeing and curing kettle (2) is completed;
S3: when the fixation process is completed, a pressure relief valve (6) is opened to relieve and the CO₂ fluid flows into a recovery kettle (3) to separate and recover CO₂.

2. The supercritical CO₂ dyeing method according to claim 1, **characterized in that** includes:
S4: after the Step S3, opening the dyeing and curing kettle (2) and taking out the object to be dyed after the fixation to wash or soap.

3. The supercritical CO₂ dyeing method according to claim 1 or 2, **characterized in that** the object to be dyed is textiles; in the Step S1, the object to be dyed is colored by means of immersion or sizing which includes: preparing a desired dyeing precursor in which one or more suitable auxiliary agents are added into, or preparing coating slurry according to different fabric materials; in the Step S2, fabrics are placed into the supercritical fluid in the dyeing and curing kettle (2) by means of a warp beam, preset process parameters includes: a pressure for fixation is 8MPa-30MPa, a temperature is 60°C to 150°C, a volume of fluid circulation in the supercritical CO₂ fluid dynamic fixation assembly is 100-1000L/h and a cycle of the dyeing process is 10min-120min; and one or more catalysts are added during the curing process in the Step S2.

4. The supercritical CO₂ dyeing method according to claim 1 or 2, **characterized in that** the object to be dyed is polyester fabrics and disperse dyes are used as dyestuffs; the Step S1 includes: adding an appropriate amount of one or more suitable thickening auxiliary agents to a dyeing precursor, immersing the polyester fabrics by means of a rolling mill, enabling the polyester fabrics to pass through the prepared precursor at a constant speed and squeezing the polyester fabrics, which is tensioned by rollers, by squeeze wheels, wherein the ratio of the dyeing precursor contained in the polyester fabrics is controlled by adjusting the pressure exerted by the squeeze wheels to 0-0.8MPa; the Step S2 includes: loading the bathed polyester fabrics on the dyeing warp beam and putting the polyester fabrics into the dyeing and curing kettle (2), opening the pressure pump (7) to pump into an appropriate amount of CO₂ into the circulation, turning on the heating jackets and the heat trace cables to heat the dyeing and curing kettle (2); when the temperature in the circulation reaches 80-140°C and the pressure reaches to 8-27 MPa which are the values of preset process parameters, turning on the circulation pump (9) at a flow rate≥20L/h; after a period of time of 10-40 min, the dye diffusion and fixation process on the polyester fabrics is completed.

5. The supercritical CO₂ dyeing method according to claim 1 or 2, **characterized in that** the object to be dyed is polyester fabrics and a method of pigment sizing is adopted to cover the polyester fabrics in the step S1; the step S1 includes: preparing suitable coating slurry, in which one or more adhesives are added into for fixation of the slurry; enabling the polyester fabrics to pass through a coating machine or a printing machine so as to uniformly apply the slurry to the polyester fabrics; the step S2 includes: loading the immersed polyester fabrics on the dyeing warp beam and putting the polyester fabrics into the dyeing and curing kettle (2), opening the pressure pump (7) to pump into an appropriate amount of CO₂ into the supercritical CO₂ fluid fixation assembly, turning on the heating jackets and the heat trace cables to heat the dyeing and curing kettle (2); when the temperature in the supercritical CO₂ fluid fixation assembly reaches 80-140°C and the pressure reaches to 8-27 MPa which are the values of preset process parameters, turning on the circulation pump (9) at a flow rate≥20L/h; after a period of time of 10-40 min, the dye diffusion and fixation process on the polyester fabrics is completed.

6. The supercritical CO₂ dyeing method according to claim 3, **characterized in that** when the object to be dyed is cotton fabrics, in the Step S2, the humidity within the supercritical CO₂ fluid dynamic fixation assembly is controlled between 40% and 90% and urea is added as a wetting agent to ensure the humidity during the curing process.

7. The supercritical CO₂ dyeing method according to claim 1 or 2, **characterized in that** the object to be dyed is textiles made of natural fibers, chemical fibers or blended fibers or textile articles, and dyes is at least one dyestuff selected from the group consisting of direct dyes, reactive dyes, cationic dyes, disperse dyes, vat dyes, azo dyes and sulfur dyes.

8. A dyeing system for the supercritical CO₂ dyeing method according to any one of claims 1-7, **characterized in that** the dyeing system comprises:
a coloring assembly including rolling mill, a coating machine or a printing machine; and
a supercritical CO₂ fluid fixation assembly, which is a supercritical CO₂ fluid dynamic fixation assembly, including:
a dyeing and curing kettle (2),
a recovery kettle (3),
a circulation connecting the dyeing and curing kettle (2) and the recovery kettle (3), which comprises a CO₂ gas cylinder (5), a pressure pump (7), a circulation pump (9) and pipelines thereamong, wherein the pressure pump (7) and a valve III (8) are disposed on a pipeline from the outlet of the CO₂ gas cylinder (5), and the outlet of the valve III (8) is respectively connected to the outlet of the dyeing and curing kettle (2) and the outlet of the recovery kettle (3) in two ways; the circulation pump (9) and a valve I (1) are disposed on a pipeline connecting the outlet of the dyeing and curing kettle (2) and the inlet of the recovery kettle (3),
a pressure relief valve (6), which is disposed on a pipeline connecting the outlet of the dyeing and curing kettle (2) and the inlet of the recovery kettle (3),
a valve II (4), which is disposed on a pipeline connecting the outlet of the CO₂ gas cylinder (5) and the outlet of the recovery kettle (3);
heating jackets, which are disposed out of the dyeing and curing kettle (2) and the recovery kettle (3), and
heat trace cables, which are wound around the pipelines connected to the dyeing and curing kettle (2) and the recovery kettle (3).

9. The dyeing system for the supercritical CO2 dyeing method according to claim 8, **characterized in that** the dyeing and curing kettle (2) has a horizontal cylindrical kettle body and the recovery kettle (3) has an elongated cylindrical kettle body in which a three-dimensional duplex filter structure is disposed.

10. The dyeing system of the supercritical CO2 dyeing method according to claim 8 or 9, wherein the coating machine employs a classic coating machine or a foam coating machine; the printing machine employs a cylinder printing machine, a flat screen printing machine or an ink jet printing machine.
